

No. 889,167.

PATENTED MAY 26, 1908.

F. WOLF.  
COMPOSITE LATHING.  
APPLICATION FILED OCT. 19, 1907.

Fig. 1.



Fig. 2.



Fig. 3.



Witnesses:

G. V. Rasmussen  
John Lotka

Inventor

FREDERICK WOLF  
By his Attorneys  
Briesen & Knauth

# UNITED STATES PATENT OFFICE.

FREDERICK WOLF, OF NEW YORK, N. Y., ASSIGNOR OF ONE-THIRD TO CARL BARKHAUSEN, OF NEW ROCHELLE, NEW YORK, AND ONE-THIRD TO GUSTAF J. BIDTEL, OF HOBOKEN, NEW JERSEY.

## COMPOSITE LATHING.

No. 889,167.

Specification of Letters Patent.

Patented May 26, 1908.

Application filed October 19, 1907. Serial No. 398,151.

To all whom it may concern:

Be it known that I, FREDERICK WOLF, a citizen of the Empire of Germany, residing in the borough of Manhattan, city, county, and

5 State of New York, have invented a certain new and useful Improvement in Composite Lathing, of which the following is a specification.

10 My invention relates to an improvement in composite lathing, which is used to hold plaster on the walls and ceilings of buildings, and is also used as a skeleton tension member in cement or concrete floors or walls.

15 In the accompanying drawings, Figure 1 is a plan view of the wire network forming the foundation of my structure. Fig. 2 is a plan view of my completed structure, and Fig. 3 a section on line 3—3 of Fig. 2.

20 In Fig. 1, *a a'*, are wires of galvanized iron or other suitable material, woven into the form of a coarse net work. The distance between the parallel wires is preferably about three quarters of an inch, although the distance may be varied to suit varying conditions.

25 In Fig. 2 the wires *a a'* are inclosed in a structure of cement which, in the particular construction shown, assumes the form of a series of crosses *c c*, surrounding openings *ff*, each cross being centered over one of the 30 points of crossing of the wires *a a'*. Each cross is preferably provided with ridges, such as ridges *d d*, and with depressions, such as depressions *e e*, to assist in holding the plaster, concrete or cement. The arms of each 35 cross are preferably gradually reduced in thickness, as at *g g*, as they approach the arms of the adjacent crosses, in order that, when the fabric is bent, either in rolling for 40 transportation or in bringing it into the shape in which it is to be used, the cement covering may easily be cracked at the thinnest portions between the arms of the crosses without injury to the main body of the covering.

45 I prefer to make the cement covering according to the following formula, although I may use any other suitable proportions or ingredients which produce a substance which may be placed about the wires in plastic form 50 and harden, without the application of fur-

nace heat, to a covering firm and strong enough to hold the plaster, concrete or cement, and not injuriously affected by the ingredients of the same.

|                                    |    |        |    |
|------------------------------------|----|--------|----|
| Calcined pulverized magnesite      | 50 | pounds | 55 |
| Solution of chlorid of magnesium   | "  | "      |    |
| (20°-25° Baumé)                    | 50 | "      |    |
| Asbestos, powder or fiber          | 30 | "      |    |
| Silex, or other silicious material | 15 | "      | 60 |

For the asbestos I may substitute cocoanut fibers, and for the silex I may substitute lava, gypsum, or ordinary cement.

I do not claim the shape of my device as new, as this is disclosed in the German patent 65 to Stauss, No. 51,158, of April 26, 1889, which describes a composite lathing in which the crosses are of brick, and are constructed by laying the clay about the wire netting and then burning it in a furnace or kiln, nor is the 70 exact shape of my lathing of importance, as long as it is provided with projections to hold the plaster, cement or concrete, it being, of course, always advisable to provide apertures, such as apertures *ff*, to enable the material to lock upon the lathing.

My composite lathing possesses particularly the merits of cheapness, lightness and durability. It is elastic and fireproof. It is lighter than "expanded metal", the amount 80 of metal being reduced to a minimum, only so much being used as is necessary to give the required strength, without employing additional metal to afford a grip for the plaster, cement or concrete; and it is more durable, 85 as all the metal is inclosed and protected by the cement covering. It is preferable to the lathing described in the above mentioned German patent for a number of reasons: The covering dries without the necessity of 90 burning in a furnace, thus making the process of manufacture a much cheaper one. The burning, besides being an expensive process, limits the size of the sheet, while my lathing may be made in strips of any length. Moreover, the burning destroys the temper of the wire and, moreover, makes the use of galvanized iron impossible, while it shrinks the clay, thus exposing portions of the wire between the ends of the crosses and such por- 95 110

tions thus becoming liable to rust. I am able to use, in my lathing, galvanized iron wire, or wire covered with rust proof paint, and even such wire practically at all times protected by the solid covering of cement.

I claim:

1. Composite lathing comprising a net work of wire covered with cement, substantially as and for the purpose described.
- 10 2. Composite lathing comprising a net work of wire covered with cement, and provided with transverse apertures, substantially as and for the purpose described.
- 15 3. Composite lathing comprising a net work of wire covered with cement of varying thickness and provided with transverse aper-

tures, substantially as and for the purpose described.

4. Composite lathing comprising a net work of wire covered with cement of varying thickness weakened at a portion substantially midway between the crossing points of the wires and provided with transverse apertures, substantially as and for the purpose described. 20 25

In witness whereof, I have hereunto set my hand in the presence of two subscribing witnesses, this 17th day of October, 1907.

FREDERICK WOLF.

Witnesses:

FRITZ V. BRIESEN,  
JOHN A. KEHLENBECK.